

# United States Patent [19]

Wells

[11] 3,753,799  
[45] Aug. 21, 1973

[54] **HEAT TREATMENT OF ALLOY STEEL PARTS**

[75] Inventor: **Kenneth Howard Wells, Solihull, England**

[73] Assignee: **Joseph Lucas (Industries) Limited, Birmingham, England**

[22] Filed: **June 1, 1971**

[21] Appl. No.: **148,747**

[30] **Foreign Application Priority Data**

Mar. 31, 1971 Great Britain ..... 8,362/71

[52] U.S. Cl. ..... **148/15.5**

[51] Int. Cl. ..... **C23c 9/14**

[58] Field of Search ..... **148/15, 15.5, 28, 148/128, 22**

[56] **References Cited**

UNITED STATES PATENTS

3,317,357 5/1967 Muller ..... 148/15.5  
1,967,994 7/1934 Malcolm ..... 148/15.5

|           |         |                 |          |
|-----------|---------|-----------------|----------|
| 2,927,875 | 3/1960  | Muller .....    | 148/15.5 |
| 3,208,885 | 9/1965  | Muller .....    | 148/15.5 |
| 3,615,908 | 10/1971 | Waterfall ..... | 148/15.5 |

**FOREIGN PATENTS OR APPLICATIONS**

|           |         |                     |          |
|-----------|---------|---------------------|----------|
| 21,868    | 10/1963 | Japan .....         | 148/15.5 |
| 1,013,712 | 12/1965 | Great Britain ..... | 148/15.5 |
| 1,052,668 | 12/1966 | Great Britain ..... | 148/15.5 |

**OTHER PUBLICATIONS**

Metals Handbook, 8th Ed., Vol. 2, 1964, pub. by ASM, pp. 129-132 & 146-149

Primary Examiner—Charles N. Lovell

Attorney—Holman & Stern

[57] **ABSTRACT**

A method of heat treating a high-chromium alloy steel part comprises maintaining the part in a fused salt mixture of cyanides and cyanates of potassium and sodium and controlling the mixture so as to maintain a desired ratio of sodium and potassium and desired proportions of cyanide and cyanate radicals.

**7 Claims, 6 Drawing Figures**

PATENTED AUG 21 1973

3,753,799

SHEET 1 OF 6



INVENTOR

*Kenneth Howard Wells*

ATTORNEYS

PATENTED AUG 21 1973

3,753,799

SHEET 2 OF 6



INVENTOR

*Kenneth Howard Wells*

ATTORNEYS

PATENTED AUG 21 1973

3,753,799

SHEET 3 OF 6



INVENTOR

*Kenneth Howard Wells*

ATTORNEYS

PATENTED AUG 21 1973

3,753,799

SHEET 4 OF 6



INVENTOR

*Kenneth Howard Wells*

ATTORNEYS

PATENTED AUG 21 1973

3,753,799

SHEET 5 OF 6



INVENTOR

*Kenneth Howard Wells*

ATTORNEYS

PATENTED AUG 21 1973

3,753,799

SHEET 6 OF 6



INVENTOR  
*Kenneth Howard Wells*

ATTORNEYS

## HEAT TREATMENT OF ALLOY STEEL PARTS

This invention relates to a method of nitriding parts formed from alloy steels.

According to the invention a method of heat treating a high-chromium alloy steel part comprises maintaining the part in a fused salt mixture including cyanides and cyanates of potassium and sodium at a temperature between 560°C and 580°C and controlling the mixture such that the ratio of potassium to sodium is between 2:1 and 1:1 and that cyanide and cyanate radicals are present as follows:-

Cyanide radicals up to 20 percent

Cyanate radicals not less than 10 percent by weights of the active components of the mixture.

The invention also resides in a process as above described when applied to a part formed of an alloy steel having percentages by weight of the following constituents.

|            |             |
|------------|-------------|
| Carbon     | 0.36-0.42   |
| Silicon    | 0.85-1.15   |
| Chromium   | 4.75-5.5    |
| Vanadium   | 0.9-1.1     |
| Molybdenum | 1.25-1.75   |
| Manganese  | 0.4 maximum |

A method according to the invention will now be described by way of example.

A fused salt mixture is prepared having the following constituents:-

|                     |
|---------------------|
| Sodium Cyanide      |
| Sodium Cyanate      |
| Potassium Cyanide   |
| Potassium Cyanate   |
| Sodium Carbonate    |
| Potassium Carbonate |

The ratio of potassium to sodium being between 1:1 and 2:1 and the percentages of active components of the bath are within the ranges: cyanide radicals up to 20 percent and cyanate radicals not less than 10 percent. The salt mixture is maintained at a temperature of between 560°C and 580°C.

Specifically the percentages of active compounds are:

Cyanide radicals 14 to 17 percent

Cyanate radicals 21 to 25 percent

The prepared mixture is placed in an alloy container having a high nickel content.

The method of the invention is particularly applicable to the treatment of spur gears for gear pumps. A spur gear is machined from a 5 percent chromium steel in the fully softened condition. The steel includes the following constituents by weight:

|            |              |
|------------|--------------|
| Carbon     | 0.36-0.42    |
| Silicon    | 0.85-1.15    |
| Chromium   | 4.75-5.5     |
| Vanadium   | 0.9-1.1      |
| Molybdenum | 1.25-1.75    |
| Manganese  | 0.4 maximum  |
| Sulphur    | 0.03 maximum |
| Phosphorus | 0.03 maximum |

The spur gear is machined so as to leave a grinding allowance and is then hardened and tempered as follows. The gear may be heated to between 1,040°C and 1,060°C either in a vacuum of between  $10^{-3}$  and  $10^{-5}$  Torr or in an atmosphere of inert gas. Alternatively and preferably the gear is heated to the above temperature in an endothermic atmosphere having a dew point of

between 30°F and 35°F. In this last case it is necessary to copper plate the gear all over before the hardening process is started.

The preferred process for copper plating includes the steps of vapour degreasing, cleaning, etching, applying a 0.0003 inch copper flash in an alkaline bath and subsequently acid copper plating to a required thickness.

When the gear has reached the required temperature (of from 1,040°C to 1,060°C) it is then cooled either in oil or in an inert gas stream. Substantially immediately thereafter, and preferably while the gear is still warm, it is heated in air for 1 hour at a temperature of between 575°C and 585°C. This last-mentioned heating takes place in a vertical forced air circulating furnace.

15 The gear is then chilled for a minimum of 1 hour at a temperature of between -60°C and -80°C and subsequently tempered for 1 hour at between 575°C and 585°C. The last heating operation also takes place in a vertical forced air circulating furnace.

20 The hardened and tempered gear is subjected to a finishgrinding operation and then cleaned by degreasing in trichloroethylene vapour and subsequently blasting with a water/air mixture in which is a suspension of white bauxilite micro powder size 400.

25 The gear is then nitrided by being placed in the fused salt mixture previously described for a minimum of 30 hours. The constituents of the salt mixture are at all times controlled so that the potassium to sodium ratio and the percentages of cyanide and cyanate radicals remained within the limits described above. This control is effected by periodic testing of samples of the mixture, and subsequent additions of salts as required to maintain the mixture within the prescribed limits.

35 There is no forced supply of oxidant to the mixture, the reactions taking place as a result of natural oxidisation.

A sample removed from the salt is dissolved in water and the carbonate present precipitated with a calcium nitrate solution. After filtration an aliquot portion of 40 the solution is titrated with a standard silver nitrate solution to two end points. The first end point, using meta cresol purple indicator gives the cyanide content and the second end point using potassium chromate gives the cyanate content.

45 A further sample is converted to chlorides of potassium and sodium by reaction with concentrated hydrochloric acid. The chlorides are dissolved in distilled water and an aliquot portion taken to which is added a solution of potassium chloride so that the final solution contains 100 parts per million of potassium. The sodium content of the solution is found by atomising in an air/acetylene flame. The sodium chloride content of the mixed chlorides can be evaluated and thus the amount of potassium chloride determined. The concentration of sodium and potassium in the original sample is thereby computed.

55 For a salt bath of known dimensions the quantities of sodium or potassium salts required to be added to the mixture to maintain it within the specified limits can be determined, an equal quantity of salt being removed from the bath prior to the addition of fresh salts. Conveniently additions of salt are made at four-hourly intervals, the quantity and type of salt added on each occasion being determined by a sample taken 1 hour previously. FIGS. 1 to 6 show graphically first approximations of the quantities of the various salts required to be added to a bath whose dimensions are 15.75 inches di-

ameter  $\times$  18 inches deep to maintain optimum percentages of cyanide and cyanate radicals.

The graphs are shown plotted for a number of constant values of the cyanate radical against varying values of the cyanide radical, both the said values being those determined from the bath samples. The quantities of salt indicated by FIGS. 1 to 3 are added if it is required to raise the sodium content of the bath, and the quantities indicated by FIGS. 4 to 6 if it is required to raise the potassium content. For example, if the sample indicates a cyanate percentage of 22 percent and a cyanide percentage of 14.4 percent the sodium content of the bath being low, the following quantities of salts are added:

|                  |        |          |
|------------------|--------|----------|
| Sodium cyanate   | 6 lb.  | (FIG. 1) |
| Sodium cyanide   | 2½ lb. | (FIG. 2) |
| Sodium carbonate | mil    | (FIG. 3) |

A further sample is taken after adding the salts, to determine the amount, if any, by which the bath constituents differ from the optimum. The differences from the optimum may be due to inaccuracies in the sampling process, intensity of working of the bath, constituents of the parts being treated, etc.

The carbonate content of the bath is determined from a sample by precipitation by the addition of a calcium nitrate solution, the carbonate being filtered out. After thorough washing with hot water, the precipitate is diluted and titrated, with dilute hydrochloric or sulphuric acid, using methyl orange indicator. When the bath has been in use for some time it may be necessary to lower its temperature to between 510°C and 530°C and to remove the carbonate-rich sludge in order to maintain the required cyanate level. After removal from the bath the gear is allowed to cool in air. Salt residues are removed with boiling water followed by scrubbing in warm water to which a detergent has been added. The white surface layer resulting from the nitriding process is chemically removed and all trace of the chemicals used in this process are themselves removed. The gear is then subjected to a further blasting with the water/air/bauxilite mixture described earlier. If at any stage in the treatment of a gear it is required to store the gear for any significant period, the gear is coated with a lanolin-based dewatering oil.

Components formed of an alloy steel of the kind described and treated by the foregoing process have been

found to possess the following characteristics:-

|                         |                           |
|-------------------------|---------------------------|
| Total etched case depth | 0.008" minimum            |
| Izod impact             | 8ft. lb. minimum          |
| Vickers hardness No:    | Core (10 Kg.) 450 minimum |
|                         | Case (2.5Kg.) 900 minimum |

Gears treated according to the method described have been found to operate satisfactorily in gear fuel pumps for petrol, the said pumps working at pressures up to 1500 pounds per square inch and temperatures up to 150°C. In these conditions there is effectively no lubrication being provided by the fuel. Wear on the gears is nevertheless within acceptable limits.

I claim:

- 15 1. A method of nitriding a high-chromium alloy steel part comprising the steps of maintaining the part in a fused salt mixture including potassium cyanide, potassium cyanate, sodium cyanide and sodium cyanate at a temperature between 560°C and 580°C for a time sufficient to effect the desired nitride case, and controlling the mixture such that the ratio of potassium to sodium is between 2:1 and 1:1 and that cyanide and cyanate radicals are present as follows:-  
Cyanide radicals 14 to 17 percent  
Cyanate radicals 21 to 25 percent by weights of the active components of the mixture.
- 20 2. A method as claimed in claim 1 the part is maintained in the mixture for approximately 30 hours.
- 30 3. A method as claimed in claim 1 in which the fused salt mixture also contains Sodium Carbonate and Potassium Carbonate.
- 35 4. A method as claimed in claim 3 in which control of said mixture includes periodic testing of samples taken from the mixture and subsequently adding to the mixture sodium and potassium salts in quantities based on the samples so as to maintain the values of the constituents of the mixture within specified limits.
- 40 5. A method as claimed in claim 4 in which said samples are tested at four hourly intervals.
- 45 6. A method as claimed in claim 4 in which said quantities of salts are added 1 hour after taking the samples on which said quantities are based.
7. A method as claimed in claim 4 which includes removing the mixture a quantity thereof equal to the total of the quantities of salts which are added.

\* \* \* \* \*